

# United States Patent Office

2,698,793

Patented Jan. 4, 1955

1

2,698,793

## SIZED PAPER COMPRISING A POLYMERIZED ALKYLENIMINE

Chester G. Landes, New Canaan, and Walter F. Reynolds, Jr., Stamford, Conn., assignors to American Cyanamid Company, New York, N. Y., a corporation of Maine

No Drawing. Application April 11, 1952,  
Serial No. 281,918

15 Claims. (Cl. 92—21)

This invention relates to the sizing of cellulosic fibers and to the formation of cellulosic felts therefrom of improved resistance to aqueous fluids. More particularly, the present invention relates to the synergistic combination of an alkaline sizing agent and an alkylenimine resin with cellulosic fibers in aqueous medium, and the formation of the thus-treated fibers into felts of improved ink and water resistance.

The manufacture of sized paper containing acid-sensitive fillers has long presented a definite problem to the art. The principal difficulty arises from the fact that the alkaline fillers commonly used, for example calcium carbonate and Raffold (calcium carbonate-magnesium hydroxide) impart an excessively high pH to the paper pulp suspensions, on the order of 8.0-9.0, whereas the size, typically sodium rosinate, can be precipitated on the fibers only under acid conditions, for example, at pH values between 4-6. It is not practical first to size the fibers under acid conditions and in a subsequent step to incorporate the carbonate filler under alkaline conditions, as under alkaline conditions the size is rapidly desorbed by the fibers resulting in the formation of paper of reduced water and ink resistance. The reverse procedure is equally impractical, as the carbonate is in substantial part destroyed by the acid, with formation of foam and bubbles, resulting in the formation of a non-homogeneous paper.

Recently, a group of cationic, hydrophobic, organic compounds has been discovered which eliminates these difficulties. These compounds are substantive to cellulose fibers in aqueous suspension, and possess the valuable property of maintaining their substantivity under the alkaline conditions required for the most effective incorporation of acid-sensitive fillers. The compounds are characterized by a cationic, hydrophilic basic nitrogenous group and by at least one long chain hydrophobic aliphatic radical containing 14-22 carbon atoms, the long chain aliphatic radical being attached to the basic nitrogenous group.

The present invention is based on the discovery that the self-polymer ethylenimine,



and of alkylenimines containing not more than four carbon atoms, in their water-soluble, hydrophilic stage, act synergistically with the above-described sizing agents. It has been found that when a small proportion of the alkylenimine resin is adsorbed by a stock of cellulosic fibers in aqueous suspension, either before or after the sizing agent has been added, and the fibers bearing both the alkylenimine resin and the sizing agent are sheeted and dried at an elevated temperature to develop the water repellent properties of the size, a paper is obtained which has a greater ink and water resistance than is afforded by the total water and ink resistance imparted by either the alkylenimine resin or the sizing agent employed separately. The cause of this surprising result is not known, and applicants do not wish to be bound by any particular theory.

2

The cellulosic sheets produced according to the process of the present invention find particular use for applications where high wet strength coupled with high water impermeability are desired. Such applications include 5 paper bags, wrapping paper, and laminating paper for the formation of cardboard and paper board useful in the manufacture of paper containers.

It is a most beneficial feature of the present invention that, so far as is known, the synergistic action of the 10 alkylenimine resin is not accompanied by any harmful effect, so that all benefits afforded the use of the sizing agents and the alkylenimine resins taken singly are retained when the two classes of materials are used in combination. Still another advantage is that no subsequent 15 treatment of the fibers is necessary, other than those inherently required to develop the sizing properties of the sizes used. A most important advantage of the present invention is that it makes it possible to reduce the consumption of sizing agents of the class described to a fraction of that previously thought necessary to produce a 20 sized paper of acceptable ink and water resistance.

It is a further important advantage of the alkylenimine 25 resins that their use does not require any adjustment in the manner in which such materials as starch, gum, wax sizes, and other organic sizing or filling agents have been previously incorporated with the fibers. We have found that from 0.1-3% or more of these additional sizing and filling agents, based on the dry weight of the paper pulp, added after the incorporation of the alkaline sizing agent 30 and the alkylenimine resin, results in still further improvement of the finished paper in water resistance and in ink resistance. Suitable starches are cornstarch, preferably cooked, potato starch, wheat starch, soya bean starch and the like. Locust bean gum, starch, and other mannogalactans may be employed, as well as casein and other proteins, preferably solubilized with borax or other alkali. In addition, any of the commercially available 35 wax size emulsions may be employed.

It is an additional advantage of the use of alkylenimine 40 resins that the water-laid sheets develop a very pronounced tackiness while they are drying. As a result, it is possible to laminate a sheet of paper produced according to the process of the present invention with an un-sized sheet of paper or paper board to yield a composite 45 paper or paper board having an adsorbent body but possessing great surface water and ink resistance. Thus a laminated blotting paper may be produced having an ink-resistant surface. It is further possible to make a well laminated cardboard of improved ply-strength by the use 50 of this intrinsic adhesiveness.

Briefly, according to the process of the present invention, small amounts of an aqueous solution or dispersion of the alkylenimine resin and an aqueous solution or dispersion of the sizing agent are separately added to a stock 55 of cellulosic fibers at any ordinary consistency in the beater. The order in which these materials is not critical, but before each addition the pH of the stock is adjusted to suitable values as discussed below, and after each addition the stock is aged until the added material has been adsorbed by the fibers. The resulting stock is sheeted 60 and dried in the normal fashion, and then is subjected to sufficient heating to develop the water-repellent properties of the size.

The alkylenimine resin is strongly bound to the fibers, 65 apparently by electrostatic forces, and cannot be leached therefrom by water. So far as is known the resin does not react or undergo further polymerization while on the fibers. The paper in its simplest embodiment thus consists essentially of cellulosic fibers, the size and the resin, both the size and the resin being uniformly distributed 70 throughout the sheet and firmly adsorbed by the fibers.

The synergistic action described above occurs to a significant degree with all commercial pulps, so that the character of the stock is not critical in the present invention. Good results have been obtained with bleached and unbleached northern kraft pulps and with a stock made 75

from corrugated boxboard containing a high percentage of sodium silicate.

In the adding the agents described, it is advantageous to maintain the pH of the pulp within the ranges at which the sizing agent and the alkyleneimine resin are respectively best adsorbed. In this respect, the sizing agents exhibit a variable behavior. All so far investigated are adsorbed very well on the acid side, for example, in the pH range of about 4 to 6. Some, however, are adsorbed on the alkaline side as well, that is, at pH values as high as 10. In the majority of cases, then, the sizing agent is added first with the stock at a pH of about 4-6. The alkyleneimine resin is added after the pH of the stock has been adjusted to a value between 8 and a pH insufficiently high to harm the fibers. A pH of 11 gives good results without harming the stock.

The alkaline sizing agents and alkylamine resins mentioned above are mutual precipitants and therefore the addition of each should be sequential and not simultaneous. Moreover, while the absorption of both classes of materials by the fibers is very rapid when the stock is maintained at respectively suitable pH values, some short period of aging is required before absorption in each instance becomes substantially complete. Ordinarily an aging period of about five minutes is ample, and a shorter time will frequently be found sufficient.

The synergistic action set forth above is very evident when as little as 10% of alkyleneimine resin is added based on the weight of sizing agent, so that there does not appear to be any lower limit to the amount of alkyleneimine resin which will produce at least some synergistic action. Maximum synergistic action appears to take place in most instances when the amount of alkyleneimine resin added is between about 1 and 3 times the weight of sizing agent. As ordinarily between about 1/2% and 5% of sizing agent is added, based on the weight of the fibers, the amount of alkyleneimine resin added will generally be at least about 1/2% of the weight of the fibers. It will be evident that much larger amounts of the alkyleneimine resin may and frequently will be added to the stock above that necessary to produce the maximum synergistic effect. Such additional amounts, which may be as high as 400% of the weight of the sizing agent or higher, are within the scope of the invention.

The alkyleneimine resins suitable for use in the process of the present invention are prepared by carefully heating monomeric ethylenimine, propylenimine, or butylenimine, or mixtures thereof in the presence of a catalyst, until polymerization has proceeded sufficiently far to form a resin which is hydrophilic and cationic but insufficiently far to render the resin hydrophobic. The end point may readily be found by testing the resin for these properties against paper pulp or by determining the viscosity of the resin as the self-condensation proceeds. A suitable resin has a viscosity of 60-120 seconds, measured by the fall time of a 3 mm. steel ball through 20 mm. of a 50% aqueous solution of the polymer at 20° C.

It is a most important feature of the invention that the use of the alkyleneimine resins does not preclude the incorporation of acid-sensitive fillers, colorants and assistants. To incorporate these materials it is only necessary, of course, that the pH of the stock is not acid at the time of addition and is not made acid at a point subsequent thereto. Thus, where the sizing agent and the alkyleneimine resin are both added with the pulp on the acid side, the stock should be made distinctly alkaline before the acid-sensitive fillers are incorporated. On the other hand, where the sizing agent is added on the acid side, and the alkyleneimine resin is added on the alkaline side, as is preferred, the fillers and colorants may be added immediately before, with, or subsequent to the incorporation of the resin.

The sizing agents are advantageously prepared from fatty amines or acids of between 14-22 carbon atom chain length. The fatty radicals may be saturated or unsaturated, but preferably will contain not more than about 50% of unsaturated molecules. In the case of fatty amines an efficient size is produced by first adding to the amine one mol of concentrated hydrochloric acid and sufficient ethanol to form a solution, then adding two mols of epichlorohydrin dropwise at 70° C., refluxing for 4 hours, and stripping off the solvent. A small amount of acetic acid may then be added to facilitate the dispersion of the product in water. Sizes are also

prepared from the fatty acid by partial acylation of a polyalkylenepolyamine. In this reaction the fatty acid and amine are mixed and heated at about 200° C. until evolution of water substantially ceases, the amount of fatty acid taken being insufficient to react with all the primary and secondary groups in the amine. An excellent product is obtained by reacting 3 mols of stearic acid with 1 mol of tetraethylenepentamine. The product is made dispersible by reaction of acid with the unreacted amine groups or by reaction of the free amine groups with one to two mols of epichlorohydrin. In this step the partially acylated polyalkylenepolyamine is suspended in an equal volume of ethanol, one to two mols of epichlorohydrin added, the mixture refluxed for 4 hours, and the solvent stripped off.

The chemical formulae of these compounds is not known, and therefore the compounds are referred to hereinafter in terms of their method of formation.

The invention will be further described by the following specific examples. Although these examples describe certain features of the invention in detail, the invention has been fully set forth above and the examples are given only for purposes of illustration and the invention is not limited thereto. Parts are by weight except where otherwise stated.

#### Examples 1-8

A slush stock was prepared from used corrugated boxboard by pulping the boxboard, passing the pulp through a refiner, and jordaning the slurry to about 600 cc. Schoepper-Riegler freeness. The pH of the resulting stock was adjusted to 10.0 with aqueous sodium hydroxide. The stock was then refined in a Morden refiner for 3 minutes, and two portions withdrawn at 2.0% fiber consistency. The pH of one of these portions was reduced to 5 by the addition of hydrochloric acid. Five aliquots were withdrawn from each of these two portions and one aliquot from each set was labelled as the control.

The pulps of the two control samples were sheeted, dried, and heated at 115° C. for 2 minutes under identical conditions, and the resulting handsheets tested for their water and ink resistance. To the remaining aliquots were added the condensation product of octadecylamine with 1.4 mols of epichlorohydrin solubilized by the addition of one mol of acetic acid as a cationic, hydrophilic ethylenimine resin, or both, as shown below in the amounts specified and in the sequences indicated. Before addition, both the size and the resin were diluted to 10% solids with water to facilitate metering.

After the addition of each of the reagents, the stock was stirred until a homogeneous mixture resulted and allowed to age 5 minutes, when absorption of the reagents was substantially complete. All the pulps were then diluted to 0.6% consistency, their pH adjusted to 10.0, and made into Nash handsheets at a basis weight (25" x 40"/500) of 47±4 pounds after a further aging period of five minutes. The percentage of ethylenimine resin in the dried paper handsheets produced by Examples 3, 4, 5, 8, 9 and 10 was determined by nitrogen analysis, allowance being made for the nitrogen content of both the control sample and the alkaline size present. The percentage of polyethylenimine in these sheets was substantially constant in the high range of 2.45% to 2.85%.

The tensile strength of the handsheets after aging for two weeks at 70° F. at 50% relative humidity were taken longitudinally and transversely and the results averaged. The water and ink resistance of the sheets were determined by the Currier and B. K. Y. methods respectively, by applying the liquids to the felt side of the sheet and noting the number of seconds required for the liquids to pass through. In the case of water, the end point was determined by an automatic electrical instrument operating by conductivity which recorded the time in seconds between the instant at which the sheets were wetted with a predetermined amount of water, and the instant at which the water penetrated. In the case of the ink, the end-point was determined by an automatic instrument employing a photoelectric cell, which recorded the time in seconds between the instant at which the ink was added to one side of the paper, and the instant at which the dark blue color of the ink appeared on the other side. In the case of the controls (Examples

1 and 6), both the water and the ink passed through the paper practically instantaneously.

## INITIAL pH OF STOCK—pH 5.0\*

| Expt. | Order of addition |         |        |         | Resistance (seconds),<br>Currier<br>B. K. Y. | Tensile<br>strength,<br>lb./in. |      |  |
|-------|-------------------|---------|--------|---------|----------------------------------------------|---------------------------------|------|--|
|       | First             |         | Second |         |                                              |                                 |      |  |
|       | Size b            | Resin b | Size b | Resin b |                                              |                                 |      |  |
| 1     |                   |         |        |         | (e)                                          | (e)                             | 17.0 |  |
| 2     | 1.5               |         |        |         | 11                                           | 60                              | 14.0 |  |
| 3     |                   | 3       |        |         | 2                                            | 40                              | 19.0 |  |
| 4     |                   | 3       | 1.5    |         | 55                                           | 1,060                           | 17.4 |  |
| 5     | 1.5               |         |        | 3       | 45                                           | 770                             | 17.4 |  |
|       |                   |         |        |         |                                              |                                 | 7.2  |  |

## STOCK AT pH 10.0 THROUGHOUT

|    |     |   |     |   |     |       |      |     |
|----|-----|---|-----|---|-----|-------|------|-----|
| 6  |     |   |     |   | (e) | (e)   | 17.0 | 0.8 |
| 7  | 1.5 |   |     |   | 10  | 60    | 14.6 | 0.8 |
| 8  |     | 3 |     |   | 2   | 45    | 18.8 | 5.4 |
| 9  |     | 3 | 1.5 |   | 61  | 1,055 | 16.8 | 6.6 |
| 10 | 1.5 |   |     | 3 | 69  | 1,320 | 16.2 | 6.6 |

\* pH raised to 10.0 immediately prior to the addition of the ethylenimine resin.

<sup>b</sup> Based on the dry weight of the fibers.

<sup>c</sup> Instantaneous.

This table shows that when only the alkaline size was added to the stock, the water resistance of the paper increased to 11 seconds, and that when only polyethylenimine was added, the water resistance increased by 2 seconds. When however, the two materials were present on the fibers in combination, the water resistance increased to 45 seconds when the alkaline size was added first and the ethylenimine resin added second with the stock at a pH of 5.0. A maximum resistance of 69 seconds was obtained when the same order of addition was followed with the stock maintained at a pH of 10.0 throughout. An even more striking increase was effected in the case of ink resistance, as the cumulative effect of the two materials employed separately was only about 100 seconds, whereas, when the two materials were employed together, the ink resistance increased to about 770 seconds in the case of experiment 5, and to 1320 seconds in the case of experiment 10.

## Example 9

A size was prepared by condensing 63 parts of tetraethylenepentamine with 199 parts of a mixture of 16-18 carbon atom fatty acids obtained by the hydrogenation of tallow at 200° C. until evolution of water had substantially ceased, and solubilizing the product with one mol of glacial acetic acid. A stock of bleached kraft pulp at 0.6% consistency was prepared, and divided into several aliquots. One aliquot was retained as control. To the second aliquot was added 1½% of the size described with the stock at pH 5.0. To the third aliquot was added 3% of cationic hydrophilic ethylenimine resin at pH 10.0. To the fourth aliquot was added first 1½% of the size followed, after 5 minutes of aging, by 3% of cationic, hydrophilic ethylenimine resin with the stock at pH 10.0. The pH adjustments were made by the use of aqueous sodium hydroxide, the size and the resin were added as 10% aqueous solutions or dispersions, and in each instance the stocks were allowed to stand until adsorption of the size and resin had become substantially complete. Handsheets were prepared from each of the four aliquots as described above and heated for 2 minutes at 115° C. to develop the water-repellent properties of the size. The sheets were conditioned at 70° F. and 50% relative humidity for two weeks and tested for their resistance to penetration by water by the Currier method. Results are as follows.

| Size added, percent | Resin added, percent | Water resistance, seconds |
|---------------------|----------------------|---------------------------|
|                     |                      | (1)                       |
| 1½                  | 3                    | 2                         |
| 1½                  | 3                    | 22                        |
|                     |                      | 30                        |

<sup>1</sup> Instantaneous.

We claim:

1. In a process for producing a sized cellulosic sheet of improved water and ink resistance, wherein ½% to 5%, based on the weight of the fibers, of a cationic, organic, water-insoluble hydrophobic sizing agent in the form of a water-dispersible salt thereof is added to a stock of cellulosic fibers in aqueous suspension, said stock is allowed to stand until adsorption of said resin is substantially complete, said fibers are formed in a sheet, and said sheet is dried and heated at a temperature between about 105° C. and 150° C. for ½ to 3 minutes to develop the sizing properties of said sizing agent, the steps of separately adding to said fibers in said medium an aqueous solution of an alkyleneimine resin in its hydrophilic, cationic stage, said resin being formed by polymerization of an alkyleneimine containing not more than 4 carbon atoms, the weight of said alkyleneimine resin being about ½ to 4 times the weight of said alkaline sizing agent, and allowing the stock to stand until adsorption of said resin is substantially complete.
2. In a process for producing a sized cellulosic sheet of improved water and ink resistance, wherein ½% to 5%, based on the weight of the fibers, of a cationic, organic, water-insoluble hydrophobic sizing agent in the form of a water-dispersible salt thereof is added to a stock of cellulosic fibers in aqueous suspension, said sizing agent being selected from the group consisting of the reaction product of a fatty amine with 1 to 2 mols of epichlorohydrin, the product formed by reacting sufficient of a fatty acid with a polyalkylenepolyamine to yield a water-insoluble amide but insufficient to acylate all of the primary and secondary nitrogen atoms in said polyalkylenepolyamine, and the reaction product thereof with 1 to 2 mols of epichlorohydrin, said stock is allowed to stand until adsorption of said resin is substantially complete, said fibers are formed in a sheet and said sheet is dried and heated at a temperature between about 105° C. and 150° C. for ½ to 3 minutes to develop the sizing properties of said sizing agent, the steps of separately adding to said fibers in said medium an aqueous solution of an alkyleneimine resin in its hydrophilic, cationic stage, said resin being formed by polymerization of an alkyleneimine containing not more than 4 carbon atoms, the weight of said alkyleneimine resin being about ½ to 4 times the weight of said alkaline sizing agent, and allowing the stock to stand until adsorption of said resin is substantially complete.
3. A process according to claim 2 wherein the resin is polymerized ethylenimine.
4. A process according to claim 2 wherein the sizing agent is the reaction product of a fatty amine with 1 to 2 mols of epichlorohydrin.
5. A process according to claim 2, wherein the sizing agent is the product formed by reacting sufficient of a fatty acid with a polyalkylenepolyamine to yield a water-insoluble amide but insufficient to acylate all of the primary and secondary nitrogen atoms in said polyalkylenepolyamine.
6. A process according to claim 2 wherein the sizing agent is the product formed by reacting sufficient of a fatty acid with a polyalkylenepolyamine to yield a water-insoluble amide but insufficient to acylate all of the primary and secondary nitrogen atoms in said polyalkylenepolyamine, and reacting the product with 1 to 2 mols of epichlorohydrin.
7. A process according to claim 2 wherein the size is added first with the stock at a pH of 4 to 6 and the resin is added subsequently when adsorption of the size is complete with the stock at a pH of 8 to 11.
8. As a new and useful composition of matter, a sheet of cellulosic fibers having uniformly adsorbed thereon between ½% and 5% of their weight of a cationic, organic, hydrophobic size selected from the group consisting of the reaction product of a fatty amine with 1 to 2 mols of epichlorohydrin, the product formed by reacting sufficient of a fatty acid with a polyalkylenepolyamine to yield a water-insoluble amide but insufficient to acylate all of the primary and secondary ni-

trogen atoms in said polyalkylenopolyamine and the reaction product thereof with 1 to 2 mols of epichlorohydrin, and 10% to 400% of an alkyleneimine resin based on the weight of the size, said sheet having been made by the process of claim 10.

10. A sheet according to claim 9 wherein the pH of the sheet is alkaline.

11. A sheet according to claim 9 wherein the resin is polymerized ethylenimine.

12. A sheet according to claim 9 wherein the size is the reaction product of a fatty amine with 1 to 2 mols of epichlorohydrin.

13. A sheet according to claim 9 wherein the size is the product formed by reacting sufficient of a fatty acid with a polyalkylenopolyamine to yield a water-insoluble amide but insufficient to acylate all of the primary and secondary nitrogen atoms in said polyalkylenopolyamine.

14. A sheet according to claim 9 wherein the size is the product formed by reacting sufficient of a fatty acid with a polyalkylenopolyamine to yield a water-insoluble amide but insufficient to acylate all of the primary and secondary nitrogen atoms in said polyalkylenopolyamine, and reacting the product with 1 to 2 mols of epichlorohydrin.

15. As a new and useful composition of matter, a laminate comprising at least one sheet corresponding to that of claim 8.

## References Cited in the file of this patent

## UNITED STATES PATENTS

|           |         |       |               |
|-----------|---------|-------|---------------|
| 2,269,997 | Berchet | ----- | Jan. 13, 1942 |
| 2,444,802 | Auten   | ----- | July 6, 1948  |
| 2,479,480 | Dudley  | ----- | Aug. 16, 1949 |